

## UNITED STATES PATENT OFFICE

2,128,621

## METHOD OF CASE HARDENING

Bernard R. Queneau, Millburn, N. J., assignor to  
 United States Steel Corporation, New York,  
 N. Y., a corporation of New Jersey

No Drawing. Application February 10, 1937,  
 Serial No. 125,157

## 8 Claims. (Cl. 148—14)

This invention relates to case-hardening steels. One object is to provide an improved case-hardened steel product. Another object is to provide an improved method of hardening case-carburized steels. Still another object is to provide a steel composition adapted to be case hardened by the practice of the thermal hardening method described and claimed in Bain et al. Patent No. 1,924,099 issued August 29, 1933. Other objects and advantages will be apparent as the invention is more fully hereinafter disclosed.

Heretofore in the art the case hardening of steels has been accomplished in the following general manner:—

15 The steel object after fabrication to its desired final size, shape and configuration is heated under surface carburizing conditions to temperatures above the critical range and maintained at this temperature for a time interval adapted to produce the desired depth to the carburized area. The thus carburized object is then rapidly cooled, as by quenching, to near atmospheric temperatures to harden the carburized area and subsequently is tempered.

20 In the practice of this "quench and temper" method of hardening the case-carburized area it has been found that in order to avoid the introduction of deleterious magnitudes of internal stresses and strains within the interior core metal 25 of the object the carbon content of the core must be maintained below about .20%. To compensate for loss in strength incident to this low carbon in the core metal it heretofore in the art has been customary to add to the steel composition 30 various so-called "toughening" constituents such as nickel, chromium, vanadium and the like. It has also been customary to incorporate various carbide-forming elements such as molybdenum, tungsten, chromium and the like for the purpose 35 of increasing the hardness of the carburized area. However, in all such alloys heretofore proposed for case-hardening purposes by the quench and temper method the carbon content of the alloy before case carburizing has been limited to about 40 .20% maximum.

I have discovered that when the case-carburized alloy is hardened by the Bain et al. method the carbon content of the alloy may be increased above .20% to as high as the eutectoid percentage 45 without introducing deleterious amounts of internal stress and strain in the hardened object and, quite to the contrary, I may obtain thereby a case-hardened article having a core evidencing very much higher load-carrying capacities than 50 heretofore obtainable and a hardened area sub-

stantially free from the hardening cracks and fissures heretofore obtained in the practice of the prior art "quench and temper" method of hardening.

I have found that the steel composition for 5 case-hardening purpose, in addition to having the higher carbon (within the range above specified) must also be varied somewhat as to associated alloy constituents with respect to the section of the object to thereby provide a composition susceptible to case hardening by the practice of the Bain et al. method.

The Bain et al. method of hardening briefly stated consists in causing austenite to undergo substantially complete transformation into stable 10 ferritic structures at some temperature within the range of temperatures below that of rapid pearlite formation and above that of rapid martensite formation. In order to accomplish this, the steel first must be heated to a temperature 15 above the critical range and converted fully into austenite and then the steel must be rapidly cooled to the temperature within this specified range at which transformation is to occur.

With any given mode of cooling as the section 20 increases the rate of heat transfer from interior to exterior decreases and consequently the time interval required to cool the major portion of the mass of the object to the desired temperature 25 thereby increases.

As indicated in Fig. 2 of the Bain et al. drawings, with any given alloy composition, for example, the plain carbon steel composition indicated, the time interval for transformation to 30 initiate at temperatures below the upper critical 35 temperature may vary widely from a few seconds to many hours depending upon the temperature. The time interval required to initiate the transformation of austenite into pearlite or into martensite is only a matter of seconds.

Therefore, a case-carburized object must be quenched at such a rate as will carry the temperature of the major mass of the metal to below the temperature of rapid pearlite formation in a 40 relatively few seconds in order to avoid the formation of relatively soft pearlite in the core metal of the case-carburized object. With objects of 45 relatively heavy section this manifestly is impractical by any known means of rapid cooling. But I have found that a very expedient way of 50 overcoming this difficulty is to incorporate in the plain carbon steel such a proportion of a transformation retarding element or elements as will extend the time of initiation of transformation to such a period of time necessary with any given 55

mode of cooling to insure that transformation will not initiate until the temperature of the major mass of the article is below the temperature of rapid pearlite formation.

5 Retarding elements found satisfactory for this purpose are nickel, chromium, molybdenum, tungsten, vanadium. These may be utilized singly or in various combinations. For example, nickel in amounts ranging from 1 to 6% has been found very effective for this purpose; and nickel-chromium in combination also has been found to be very effective, in which case nickel in amounts ranging from 1 to 4% and chromium in amounts ranging from 0.25 to 2% may be used. The specific amount of the transformation retarding element incorporated in the alloy may be varied widely without departure from my invention depending upon the section of the article and upon the extent to which the benefit thereof on the 10 core metal is desired.

15 To obtain the maximum benefit the entire core metal should be protected against pearlite formation. In very heavy sections this may not be either desirable or necessary and accordingly the 20 specific amount of the retarding agent incorporated need be only that required to insure the transformation of a desired mass of the core into ferritic structures other than pearlite and martensite at the quench temperature.

25 30 In association with the transformation retarding element I may utilize one or more of the elements (chromium, molybdenum, tungsten, vanadium) heretofore recognized in the art as benefiting the carburized area either as toughening or hardening agents. These elements in part singly or in combination with or without nickel or manganese also function as retarding elements as hereinabove discussed. Accordingly, in the broadest aspect the present invention comprises 35 40 a case-carburizing steel consisting (1) of a plain carbon steel having a carbon content above .20% and not in excess of the eutectoid percentage; (2) of the same steel plus a proportion of a transformation retarding agent or agents adapted with 45 any given mode of cooling to give a time interval of initiation of transformation at least sufficient to permit cooling of the major mass of the steel to below the temperature of rapid pearlite formation and the case-carburized area down to the 50 desired hardening temperature, which hardening temperature preferably is within the lower temperatures of the range defined in the Bain et al. patent; and (3) either alloy composition of (1) and (2) above containing a proportion of an 55 alloy constituent adapted to benefit by hardening or toughening or both, the case-carburized area of the steel.

60 As a specific embodiment of the practice of the present invention, a plain carbon steel (as defined in (1) above) having a carbon content above .20% and not in excess of the eutectoid percentage may be case carburized in accordance with prior art practice and may be case hardened by the practice of the method of the Bain et al. 65 patent, in sections up to  $\frac{1}{2}$ " thickness without the formation of substantial amounts of pearlite in the center core member. As an example,  $\frac{1}{2}$ " square bars of plain carbon steel containing .64% carbon may be case hardened by quenching from 70 the carburizing temperature down to about 400° F. in a molten salt bath and maintained at this temperature for a period of about 5 hours. Such a case-hardened steel will evidence a maximum outer fibre stress of about 312,000 pounds per 75 square inch as compared to about 68,000 pounds

per square inch when the same steel is quenched and tempered in accordance with prior art practice. This indicates the relatively higher load-carrying capacity of the case-hardened steel of the present invention over that obtainable by prior practice. 5

As a comparison, the load-carrying capacity of this .64% carbon steel hardened by the Bain et al. method was over twice that of a typical low carbon nickel-chrome case-hardening steel of the 10 same section hardened by the quench and temper method.

15 In addition to this advantage of higher load-carrying capacity, the hardened case by reason of the fact that martensite formation is avoided in the thermal hardening method, is superior physically to the case obtained by the quench and temper method. The superiority is evidenced by the fact that shallower cases may be employed and that re-grinding costs are reduced to a 20 minimum.

25 Where the section and size of the article is in excess of that permitting relatively rapid quenching of the article down to the desired hardening temperature (for example, 400° F.) 30 various alloying percentages of manganese, nickel, chromium or nickel and chromium, manganese and chromium, may be incorporated in the plain carbon steel to retard the transformation of austenite into ferrite for a sufficient time interval 35 to permit such cooling.

35 For example, nickel about 3.5% will retard transformation about five (5) seconds, while nickel 1.25% and chromium .65% will retard transformation about forty (40) seconds. With 40 this latter combination (Ni.Cr) I am enabled to successfully case harden objects having a thickness of one inch at 400° F. as above described and prevent the core metal from undergoing transformation into pearlite obtaining instead ferritic structures stable at temperatures intermediate the temperatures of rapid martensite and rapid pearlite formation but higher than 45 400° F.

Having broadly and specifically described the 45 present invention and given several specific embodiments thereof, it is apparent that many modifications may be made without departing essentially from the nature and scope of the invention as may be included within the following 50 claims.

What I claim is:

1. The method of hardening a steel article 55 comprised of carbon steel containing the usual amounts of Mn, Si, S and P and containing carbon in excess of .20% but not more than the eutectoid percentage, the marginal areas of said article containing a higher carbon content than the central or core area of the article, which comprises rapidly cooling the article from a temperature above the upper critical temperature at which the said steel is fully austenitic to a temperature below the temperature of rapid pearlite formation but above the temperature of rapid martensite formation and holding the said 60 article at a temperature within the lower portion of this said range until the austenite has undergone substantially complete transformation into ferritic structures other than martensite which are stable at the said holding temperature, 65 and then cooling to atmospheric temperatures. 70

2. The method of claim 1, the said holding temperature approximating but above about 400° F.

3. The method of claim 1, the said rapid cool- 75

ing being at a rate adapted to lower the temperature of the major proportion of the mass of the article to below the temperature of rapid pearlite formation before transformation of the austenite into ferritic structures initiates.

5. The method of claim 1, in which the said steel composition is modified by incorporating within the carbon steel, prior to forming the said article, a proportion of a transformation 10 retarding element consisting of at least one of the elements Mn, Cr, Ni, W, Mo and V in an amount sufficient to retard the initiation of transformation during rapid cooling for a time interval adapted to permit the cooling of the 15 greater proportion of the mass of the article to temperatures below the temperature of rapid pearlite formation with the mode of cooling employed.

5. In the case hardening of steel containing 20 carbon in excess of .20% but not over the eutectoid percentage, the method which comprises case carburizing the said steel at a temperature above the upper critical temperature and rapidly cooling the case-carburized product from the 25 carburizing temperature to a temperature approximating but above about 400° F. and holding the said steel at this said temperature for a time interval adapted to permit the said steel to undergo transformation from austenite into 30 ferritic structures other than martensite which are stable at the temperature of holding, and then cooling the steel to atmospheric temperatures.

6. In the case hardening of steel containing 35 carbon in excess of .20% but not over the eutectoid percentage and a proportion of a transformation retarding element of the group consisting of Mn, Cr, Ni, W, Mo and V, which comprises case carburizing the steel at a tempera- 40 ture above the upper critical temperature, cool-

ing the article from the carburizing temperature to a temperature below the temperature of rapid pearlite formation at a rate sufficient to cool the major proportion of the mass of the steel to below the temperature of rapid pearlite 5 formation before transformation initiates, interrupting the cooling of the steel before any portion of the mass has cooled to below about 400° F., and holding the temperature of the steel at temperatures approximating but above 10 400° F. for a time interval adapted to permit substantially complete conversion of the austenite into ferritic structures stable at the holding temperatures, and then cooling to atmospheric temperatures. 15

7. An article of manufacture comprised of steel containing the usual percentages of Mn, Si, S and P common to case-hardening steel but containing carbon in the core metal in amounts ranging from above .20% to the eutectoid percentage, the said article having been case carburized and hardened by the method of claim 1. 20

8. An article of manufacture comprised of steel containing the usual percentages of Si, S and P common to case-hardening steel but containing carbon above .20% but not over the eutectoid percentage and a proportion of a transformation retarding agent consisting of at least one of the metals of the group Mn, Cr, Ni, W, Mo and V, in an amount adapted to retard the 25 initiation of transformation of austenite into pearlite for a time interval sufficient to permit the cooling of the major portion of the mass of the article from a temperature above the upper critical temperature to a temperature below the 30 temperature of rapid pearlite formation, the said article having been case carburized and hardened by the method of claim 5. 35

BERNARD R. QUENEAU. 40